

(No Model.)

C. L. COFFIN.  
METHOD OF ELECTRIC WELDING.

No. 425,164.

Patented Apr. 8, 1890.



Witnesses  
Cyrus L. Coffin  
Henry Blockley

Inventor  
Charles L. Coffin.

# UNITED STATES PATENT OFFICE.

CHARLES L. COFFIN, OF DETROIT, MICHIGAN.

## METHOD OF ELECTRIC WELDING.

SPECIFICATION forming part of Letters Patent No. 425,164, dated April 8, 1890.

Application filed November 6, 1889. Serial No. 329,394. (No model.)

*To all whom it may concern:*

Be it known that I, CHARLES L. COFFIN, of Detroit, in the county of Wayne and State of Michigan, have invented a new and useful 5 Improvement in Electric Welding, of which the following is a specification.

My invention consists in a process of electric welding, hereinafter fully described and claimed.

10 Figure 1 is a perspective of an apparatus which may be used to practice my invention, and Fig. 2 is a vertical central section through the apparatus for re-enforcing a weld.

15 G represents a table, of wood or other insulating material, provided with clamps M N, having set-screws P O, and connected by the conductors F Q with the opposite poles of a generator of electricity.

20 H H represent two articles to be welded together, laid on table G with their welding edges in contact and secured by the set-screws in the clamps M N.

A represents a conductor connected with F and with a binding-screw B on a conductor K, 25 the end of which may terminate in a roller J, as shown, or may be a simple flat or rounded end. Resistance-coils A' and F' are located in the conductors for the purpose of directing the bulk of the circuit through either conductor at will, and more particularly for forming 30 a voltaic arc between the points K and H H, as more particularly hereinafter described.

E is an insulating-handle on conductor K. 35 T T represent two insulated rollers on the ends of arms I I, which branch from the conductor K, and their purpose is to facilitate carrying the lower end on conductor K along the joint, either in contact with or at a slight 40 distance from H H. By placing the rollers T T out of line the lower end of K (the roller J, as shown) tilting the conductor will throw it in or out of contact with H H.

D represents a hollow conductor (carbon) 45 carried on an insulating-handle E, connected with the conductor A, and C represents a wire or rod of metal like H H, passing down through conductor D. This is used when an irregularity, such as is shown at L, Fig. 2, is en-

countered in the welding edges of H H, the 50 rod C melting and re-enforcing the joint at L.

My process is carried out as follows: H H being placed as shown in Fig. 1, the electric current is established through conductor F, clamp N, articles H H, clamp M, and conductor Q, thus heating the edges of H H. The lower end of conductor K (roller J) is now brought in contact with the meeting edges of H H, thus shunting a part of the current through conductors A and K and increasing 60 the local heating effect of the current of the edges of H H, and conductor K is traversed along said joint. An increased heating effect may be produced by bringing conductor K into contact with H H, thus establishing the 65 circuit, then slightly raising conductor K, whereby a voltaic arc is formed between K and H H, and traversing the joint with the arc. If an irregularity like L is encountered, the conductor D is substituted for conductor 70 K, and enough of wire C to fill the hole L is melted by the voltaic arc. When the edges of H H are brought to a welding heat, the weld is formed by pressing H H together, and may be finished by rolling, hammering, or in any 75 other known way.

What I claim as my invention, and desire to secure by Letters Patent, is—

1. The herein-described process of welding metals electrically, consisting in placing the 80 articles to be welded in contact, connecting them with opposite poles of a generator of electricity, passing a heating-current through them, simultaneously traversing the joint with an electric conductor, one end of which 85 is connected with one pole of the generator and the other end in contact with the joint, and finally completing the weld by pressure.

2. The herein-described process of welding metal electrically, consisting in placing the 90 articles to be welded in contact, connecting them with opposite poles of a generator of electricity, passing a heating-current through them, simultaneously traversing the joint with a voltaic arc sprung between the joint 95 and a conductor connected with one pole of the generator, and finally completing the weld by pressure.

3. The herein-described process of welding metal electrically, consisting in placing the articles to be welded in contact, connecting them with opposite poles of a generator of 5 electricity, passing a heating-current through them, simultaneously traversing the joint with a voltaic arc sprung between the joint and a conductor connected with one pole of

the generator, re-enforcing the joint by supplying like metal carried by the traversing conductor and fused by the arc, and finally completing the weld by pressure.

CHARLES L. COFFIN.

Witnesses:

CYRUS E. LOTHROP,  
GERTRUDE ANDERSON.